

# United States Patent Office

3,193,407

Patented July 6, 1965

1

3,193,407

## FINISHED POLYOLEFIN FIBERS AND METHOD OF PREPARATION

Ann S. Keller, Norristown, and Harry H. Hall, Springfield, Pa., assignors, by mesne assignments, to FMC Corporation, San Jose, Calif., a corporation of Delaware

No Drawing. Filed Apr. 19, 1962, Ser. No. 188,865  
10 Claims. (Cl. 117—138.8)

This invention relates to finished polyolefin fibers. More particularly, it relates to polyolefin yarns or fibers having applied finishes which enable the yarns to be satisfactorily processed and utilized in the commercial production of textiles and in machine sewing operations.

Polyolefin yarns, for example polypropylene and polyethylene yarns, tend to develop high electrostatic charges and excessive tensions when running over guides, godets, and other objects during processing and subsequent handling. The utilization of unfinished polyolefin yarn in textile production and sewing equipment is unsatisfactory.

Static and tension problems have been encountered in the use of other natural and synthetic polymer yarns, and finishes which are satisfactory from both the standpoints of application and use have been developed for them. However, the polyolefins have different physical characteristics than most other filament forming polymers and conventional finishes and methods for application thereof are not suitable or effective in providing the necessary fiber to fiber lubrication, proper fiber to metal frictional behavior, and adequate static suppression.

A primary object of this invention is to provide a finished polyolefin yarn which is suitable for high speed processing, textile and sewing operations.

It is another object of this invention to provide a method of finishing polyolefin fibers which is effective in providing fiber lubrication and static suppression.

These and other objects are accomplished in accordance with this invention with a polyolefin yarn including polyethylene, polypropylene and polyisobutylene yarn having incorporated thereon a finish consisting of from 3 to 12% by weight of a morpholine derivative of the following general formula



wherein R is an alkyl sulfate having 1 to 2 carbon atoms, R' is an aliphatic hydrocarbon radical having from 12 to 30 carbon atoms and R'' is an alkyl radical having 1 to 2 carbon atoms, and a lubricant selected from the group consisting of fatty acid monoesters of polyethylene glycols wherein the fatty acid has from 12 to 18 carbon atoms and the polyethylene glycol has an average molecular weight of from about 200 to 600 and glycerol trioleate.

The method of preparing finished polyolefin yarn comprises applying to said yarn the above-described finish composition in the absence of water and a hydrocarbon oil.

The morpholine derivative of this invention is a known antistat for synthetic fibers applied in a mineral oil vehicle or carrier. The compounds include for example N-cetyl N-ethyl morpholinium ethosulfate; N-cetyl N-methyl morpholinium methosulfate; N-lauryl N-ethyl morpholinium ethosulfate; N-stearyl N-ethyl morpholinium ethosulfate; N-soyaryl N-ethyl morpholinium ethosulfate; etc.

The fatty acid monoesters of polyethylene glycols having molecular weights of at least about 200 up to about 600 provide excellent lubricity for the polyolefin fibers in multifilament, monofilament and staple form when applied dry, i.e., without water or mineral oil. Examples of these lubricants include the oleic acid monoester of polyethyl-

2

ene glycols having molecular weights respectively, of about 200, about 400, and about 600; the lauric acid monoester of polyethylene glycols having molecular weights respectively of about 200, about 400 and about 600; the stearic acid monoester of polyethylene glycols having molecular weights respectively of about 200 and about 400; the palmitic acid monoester of polyethylene glycols having molecular weights respectively of about 200, about 400 and about 600; etc.

10 The finishes of this invention may be applied to the fiber by any known means including bath, spray, padding, kiss roll application or the like.

Many lubricant-antistat combinations were investigated to develop a satisfactory finish composition for polyolefin fiber. Before combinations of lubricants and antistats were tried, however, a screening test was conducted to determine whether the lubricant or antistat material would degrade the polyolefin. Screening involved placing approximately 0.2 ml. of the liquid lubricant or antistat onto a sheet of polypropylene film which had been secured to a glass plate. A piece of graph paper was placed between the film and the glass and served two purposes; it would indicate penetration of the film by the liquid, and also give an indication of the spreading action of the lubricant or antistat. The material passed the screening test if twenty-four hours of film contact produced no change in film appearance such as waviness or puckering. If puckering did occur it was assumed that it was caused by penetration of the lubricant or antistat into the film and this type of behavior would also occur with a polypropylene fiber. Puckering was considered to be caused by plasticization or a similar phenomenon and test materials causing it were rejected.

The above screening test indicated that paraffinic oils 35 and low molecular weight esters had a noticeable undesirable effect on the test film. Application of these materials to polyolefin yarn at spinning and the consequential softening or plasticization of this yarn corroborated the screening test results.

40 To demonstrate the specificity of this invention there is set forth in the following table a list of finishes the components of which have passed the screening test but which have been found unsatisfactory either in their application or in their ability to improve the characteristics of the 45 yarn.

TABLE I

| No. | Finish composition                                    | Percent by weight |
|-----|-------------------------------------------------------|-------------------|
| 50  |                                                       |                   |
| 1   | Diethyl cyclohexylamine salt of lauryl sulfate        | 3-5               |
| 2   | Coconut oil                                           | 95                |
| 3   | Diethyl cyclohexylamine salt of lauryl sulfate        | 3-10              |
| 55  | Sorbitan monooleate                                   | 1.5-5             |
| 4   | Butyl stearate                                        | 85-95.5           |
| 5   | Diethanolamine salt of dioauryl phosphate             | 3                 |
| 6   | Sorbitan monooleate                                   | 4                 |
| 7   | Butyl stearate                                        | 93                |
| 60  | 1-hydroxyethyl-2-oleyl ethyl glyoxolinium ethosulfate | 3                 |
| 8   | Sorbitan monooleate                                   | 3                 |
| 9   | Butyl stearate                                        | 94                |
| 10  | 1-hydroxyethyl-2-oleyl ethyl glyoxolinium ethosulfate | 5                 |
| 11  | Sorbitan monooleate                                   | 95                |
| 12  | 1-hydroxyethyl-2-oleyl ethyl glyoxolinium ethosulfate | 3                 |
| 65  | Sorbitan trioleate                                    | 4                 |
| 13  | Esterified pentaerythritol                            | 20                |
| 14  | Diethyl cyclohexylamine salt of lauryl sulfate        | 75                |
| 15  | Water                                                 | 10                |
| 16  | Diethyl cyclohexylamine salt of lauryl sulfate        | 90                |
| 17  | Diethylene glycol                                     | 10                |
| 18  | Diethyl cyclohexylamine salt of lauryl sulfate        | 90                |
| 19  | Polyethylene glycol (M. W. 400) monooleate            | 5                 |
| 20  | Diethyl cyclohexylamine salt of lauryl sulfate        | 95                |
| 21  | Dialiphatic ether of polyethylene glycol              | 5                 |
| 22  | Esterified pentaerythritol                            | 95                |
| 23  | Nonionic emulsifying agents                           | 60                |
| 24  |                                                       | 40                |

TABLE I—Continued

| No. | Finish composition                                 | Percent by weight |
|-----|----------------------------------------------------|-------------------|
| 13  | Finish No. 12                                      | 10                |
|     | Water                                              | 90                |
| 14  | Finish No. 12                                      | 95                |
|     | Sorbitan monooleate                                | 3                 |
| 15  | N-cetyl N-ethyl morpholinium ethosulfate           | 2                 |
|     | Finish No. 14                                      | 20                |
|     | Water                                              | 80                |
| 16  | N-cetyl N-ethyl morpholinium ethosulfate           | 5                 |
|     | Technical grade octanol                            | 95                |
| 17  | N-cetyl N-ethyl morpholinium ethosulfate           | 10                |
|     | Water                                              | 90                |
| 18  | N-cetyl N-ethyl morpholinium ethosulfate           | 10                |
|     | Diethylene glycol                                  | 90                |
| 19  | N-cetyl N-ethyl morpholinium ethosulfate           | 2                 |
|     | Finish No. 12                                      | 98                |
| 20  | Polyoxyethylene modified tallow acid primary amine | 5                 |
|     | Polyethylene glycol (M.W. 200) monolaurate         | 95                |
| 21  | Polyethylene glycol (M.W. 200) monopalargonate     | 100               |
| 22  | Polyethylene glycol (M.W. 1000) monostearate       | 2                 |
|     | Polyethylene glycol (M.W. 200) monopalargonate     | 98                |
| 23  | Polyethylene glycol (M.W. 400) monopalmitate       | 2                 |
|     | Diethanolamine salt of dilauryl phosphate          | 95                |
| 24  | Finish No. 22                                      | 10                |
|     | Diethanolamine salt of dilauryl phosphate          | 90                |
| 25  | Polyethylene glycol (M.W. 200) monopalargonate     | 2                 |
|     | Polyethylene glycol (M.W. 400) monopalmitate       | 98                |
| 26  | Water                                              | 10                |
|     | Diethanolamine salt of dilauryl phosphate          | 90                |
|     | Polyethylene glycol (M.W. 200) monolaurate         | 90                |

In addition to the above yarn finish compositions, many other unsatisfactory combinations were tested which were identifiable only under chemical tradenames and/or broad chemical terms.

Polyolefin fibers and in particular polypropylene fibers are much more difficult to finish than other synthetic or natural polymer fibers. They are non-polar materials and as such have no affinity for yarn finishes. They are hydrophobic and, in general, water based finish compositions cannot be used to obtain a satisfactory finish. The polyolefin fibers are degraded by treatment with hydrocarbon oil base compositions and become undesirably soft. For these reasons the method of finish application and finish composition are extremely critical in order to obtain satisfactory yarn characteristics.

The following examples are set forth to demonstrate finish application and compositions in accordance with the invention.

#### Example I

A finish was prepared by mixing together 5% by weight of N-cetyl N-ethyl morpholinium ethosulfate and 95% by weight of the oleic acid monoester of polyethylene glycol of an average molecular weight of about 400. The finish was applied to newly melt spun polypropylene multifilament approximately 800 denier, 34 filament yarn just prior to primary take-up by means of a kiss roll applicator 6 inches in diameter and 1½ inches wide. The yarn was collected on a standard take-up tube without difficulty. In further processing such as draw-twisting, no difficulty with the yarn was observed.

The above procedure was also carried out with a finish consisting of 10% by weight of the same morpholinium compound and 90% by weight of the same polyglycol ester, but the finish failed to provide satisfactory processing characteristics for the yarn. This demonstrates that component amounts for the composition are also critical.

#### Example II

A yarn finish was prepared by mixing together 5% by weight of N-cetyl N-ethyl morpholinium ethosulfate and 95% by weight of the lauric acid monoester of polyethylene glycol of an average molecular weight of about 75

The finish was applied to the melt spun yarn in the same manner described in Example I. The finished yarn was processed in the usual fashion without demonstrating any difficulties caused by static or excessive tension.

As in Example I the proportions of the components of the finish were changed to 10% morpholinium derivative and 90% polyglycol ester. The finish was found to be unsatisfactory in supplying the necessary antistatic and friction properties to the yarn.

#### Example III

A yarn finish was prepared by mixing together 5% by weight of N-cetyl N-ethyl morpholinium ethosulfate and 95% by weight of glycerol trioleate. This finish was applied to the yarn as described in Example I. The finished yarn was processed as usual without experiencing any difficulties caused by static or excessive tension.

Various changes and modifications may be made in practicing the invention without departing from the spirit and scope thereof and, therefore, the invention is not to be limited except as defined in the appended claims.

We claim:

1. Polyolefin fibers having incorporated thereon a finish consisting of 3 to 5% by weight of a morpholine derivative of the following general formula:



30 wherein R is an alkyl sulfate having 1-2 carbon atoms, R' is an aliphatic hydrocarbon radical having from 12-30 carbon atoms and R'' is an alkyl radical having 1-2 carbon atoms and from 97 to 95% by weight of a lubricant selected from the group consisting of fatty acid monoesters of polyethylene glycol wherein the fatty acid has from 12-18 carbon atoms and the polyethylene glycol has an average molecular weight of from about 200 to about 600 and glycerol trioleate.

35 2. The fibers of claim 1 which is polypropylene.

3. The fibers of claim 1 wherein the morpholine derivative is N-cetyl N-ethyl morpholinium ethosulfate.

4. The fibers of claim 1 wherein the lubricant is the oleic acid monoester of a polyethylene glycol.

45 5. The fibers of claim 1 wherein the lubricant is the lauric acid monoester of a polyethylene glycol.

6. The fibers of claim 1 wherein the lubricant is glycerol trioleate.

50 7. A method of preparing finished fibers which comprises treating polyolefin fibers with a finish in the absence of water and hydrocarbon oil, said finish consisting of from 3-5% by weight of a morpholine derivative having the following general formula:



60 wherein R is an alkyl sulfate having 1-2 carbon atoms, R' is an aliphatic hydrocarbon radical having 12-30 carbon atoms and R'' is an alkyl radical having 1-2 carbon atoms, and from 97 to 95% by weight of a lubricant selected from the group consisting of fatty acid monoesters, polyethylene glycols wherein the fatty acid has from 12-18 carbon atoms and the polyethylene glycol has an average molecular weight of from about 200 to about 600 and glycerol trioleate.

65 8. The method of claim 7 wherein polypropylene fibers are treated with a finish consisting of N-cetyl N-ethyl

morpholinium ethosulfate and the oleic acid monoester of a polyethylene glycol.

9. The method of claim 7 wherein polypropylene fibers are treated with a finish consisting of N-cetyl N-ethyl morpholinium ethosulfate and the lauric acid monoester of a polyethylene glycol.

10. The method of claim 7 wherein polypropylene fibers are treated with a finish consisting of N-cetyl N-ethyl morpholinium ethosulfate and glycerol trioleate.

References Cited by the Examiner

UNITED STATES PATENTS

- |             |       |                      |           |    |
|-------------|-------|----------------------|-----------|----|
| 2,690,426   | 9/54  | Jefferson et al. --- | 117—139.5 | XR |
| 2,695,270   | 11/54 | Jefferson et al. --- | 117—139.5 | XR |
| 5 3,009,830 | 11/61 | Levine -----         | 117—139.5 | XR |

WILLIAM D. MARTIN, *Primary Examiner.*

RICHARD D. NEVIUS, *Examiner.*